

Aug. 26, 1930.

R. L. GILLISPIE

**1,774,263**

## RAILWAY TRACK STRUCTURE

Filed Dec. 22, 1928 3 Sheets-Sheet 1



Inventor

*R. L. Gillispie.*

234 R. S. C. Dougherty.  
Attorney

Aug. 26, 1930.

R. L. GILLISPIE

1,774,263

RAILWAY TRACK STRUCTURE

Filed Dec. 22, 1928 3 Sheets-Sheet 2



By *R. S. C. Wougherty.*  
Attorney

Aug. 26, 1930.

R. L. GILLISPIE

**1,774,263**

## RAILWAY TRACK STRUCTURE

Filed Dec. 22, 1928 3 Sheets-Sheet 3

*Fig. 12.*



Inventor:

*R.L. Gillispie.*

334 R. S. C. Longhena, Attorney

## UNITED STATES PATENT OFFICE

RAYMOND L. GILLISPIE, OF STEELTON, PENNSYLVANIA, ASSIGNOR TO BETHLEHEM STEEL COMPANY

## RAILWAY-TRACK STRUCTURE

Application filed December 22, 1928. Serial No. 327,768.

This invention relates to track structures, such as frogs and crossings, which comprise rail members integral with a center piece.

It is old to prepare structures of this general sort by casting the main body of the center piece in such a way as to embed the ends of the rail members therein, thus effecting an integral union of the rail members and center piece. In the cast portion of such structures a depression or pocket is formed at the intersection point of the gage lines, and into this depression is fitted a center plate having wearing qualities superior to those of the rails. Various methods have been employed to secure the center plates in position. A common practice has been to fit the plate in a pocket provided for that purpose and secure it in place by means of bolts or wedges and fill the space between the hard center and the walls of the pocket with a soft metal alloy. Another practice has been to make the center plate an integral part of the track structure by casting a metal body around the ends of the rail members and the center plate. Another common practice has been to cast a wear resisting center comprising a body portion provided with integral arms to which the track rails are bolted.

It is old to make track structures having rail members integral with the center piece by casting such structures entire, that is to say, by directly casting the whole structure, rail members as well as center piece; the whole structure thus being a single casting.

My invention is based upon the idea of first forming a center piece and then securing rail members thereto in such a way as to form an integral union therebetween.

More particularly, my invention comprises a track structure having a cast center piece and rolled rail members welded thereto.

Herein it is desired to set forth a specific embodiment for the purpose of illustrating the invention.

Referring to the accompanying drawings: Fig. 1 is a plan view of the frog center with the rail members welded thereto;

Fig. 2 is a side elevation of the weld between the end of a rail and the frog center;

Fig. 3 shows the undercut at the end of

the web of the frog center under the head portion;

Fig. 4 is a section taken on the line 4—4 of Fig. 1;

Fig. 5 is a section taken on the line 5—5 of Fig. 4;

Fig. 6 is a plan view of the finished frog;

Fig. 7 is a side elevation of Fig. 6;

Fig. 8 is a sectional view of the frog center taken on the line 8—8 of Fig. 9;

Fig. 9 is an end section taken on the line 9—9 of Fig. 6;

Fig. 10 is an end section taken on the line 10—10 of Fig. 6;

Fig. 11 is an end section taken on the line 11—11 of Fig. 1; and

Fig. 12 is a view of the rail members abutting a frog center prior to welding and showing the cutaway portions at the ends of the rails.

Rail members 14 are welded to the cast frog center 15 to make a complete frog. Rails 14 are of the rolled grooved rail type and comprise a base flange 16, web 17, head 18, and a guard flange 19. The head and guard flange are separated from each other by a groove or flangeway 20, in which the flange of the car wheel is adapted to travel.

The cast center is preferably made of alloy steel hardened by heat treatment and having wearing qualities superior to those of the rolled rails and comprises base flanges 21 which serve as spiking ledges, vertical webs 22, head or tread portion 23, and guard flanges 24. The head and guard flanges are separated from each other to form a groove or flangeway 25 in which the flange of a car wheel travels. The cross section at the ends of the cast center is practically the same as that of the rail.

Cross webs 26 between the vertical webs, and outside webs 27 are provided to stiffen the whole structure and act as gussets. The table portion 28 is raised above the normal height of the rail grooves 20 at the point of intersection and gradually tapers down towards the ends to the normal depth of the grooves of the connecting rails

so that a car wheel when approaching an intersection in a track structure will have its tread elevated above the face of the head 100

of the rail to eliminate pounding and wear due to the wheel tread passing over the interrupted rail heads at the intersection.

The frog or crossing center is of the same height as the abutting rails, getting its support directly from the ties and track substructure, thereby lessening the chances of becoming loosened from the rest of the structure. The center piece abuts the ends of the rails at the top portion only, the webs 22 and flanges 21 being undercut to provide a clearance 29 between the webs of the center and the webs of the rails for a purpose hereinafter explained. The ends of the center are cut to the corresponding angles of the rail ends and converge to a point intermediate the heads of the rails. The top sides 30 of the center are straight, the length and direction of these lines being determined by the outside lines 20 of the guard portions 19 of the rails and upon the angle of the structure. The outside lines of the base flanges are determined in a similar manner.

Prior to welding the center piece to the rail members, the ends of the rails and the ends of the center are cut to the correct angle and the guard portions 19 at the ends of the rails are cut away as shown at 31 to provide a clearance between the ends of the rails and the center. These cuts together with the undercuts 29 at the ends of the vertical webs 22 provide spaces between the pieces to be joined for the welding material. Similar spaces 32 are provided between the base flanges 21 of the center and the base flanges 16 of the rails.

The welds are preferably made by the well known thermit process in which the rails and center are set up about six inches above the bed, leveled, aligned and clamped in place. The rail ends and center are then warmed with a torch and heated wax is roughly applied by hand over the joints and then trimmed and smoothed to conform to the desired finished welds 33. The parts to be welded are then ready for the box and sand moulding commonly employed in this process. The box is set in place and as the sand moulding progresses, the heating gate cores, pouring gate cores and risers are set in place. The mould is vented and is ready for preheating which may be done by means of a large blow torch or other suitable means. The wax forms are mostly consumed in the preheating and very little runs out of the mould. The heating gates are then plugged and the mould is ready for pouring. After the preheating the thermit is melted in a crucible and in a brief time is ready for pouring into the mould. After pouring, the mould is left to cool and the frog is taken out and cleaned and the gates burned off. The welds are then planed off level with the head or guard of the rail, the bottom finished likewise, and 65 the flangeways planed out as shown in Fig.

6. Obviously it is not essential that the bottom weld be planed off. In fact the weld is stronger when not planed off.

While mitred joints are here shown between the rail member and the casting, it is 70 obvious that other forms may be used, as for example, square joints.

As stated above it is desired to make the center piece of such metal and so heat treat it as to produce wearing qualities in the center 75 piece superior to those of the rails. Steels somewhat high in silicon have been found to be very effective for the cast center pieces. The following steels have been found to be suitable for this purpose:

|            |      |      |      |
|------------|------|------|------|
| Carbon     | 55   | to   | 70   |
| Manganese  | 70   | to   | 1.00 |
| Phosphorus | 04   | Max. |      |
| Silicon    | 1.90 | to   | 2.20 |

The center pieces cast from these steels are 85 preferably heat treated, as for example, in the following manner: After cleaning they are heated to a temperature of about 1500° F. and are then quenched in oil, being allowed to remain in the oil bath until their temperature 90 is well below the critical range, say about 700° F. The length of time of quench will vary, depending upon the size of the casting. Following the quenching operation the cast 95 center piece is placed in a furnace and re-heated to a temperature of the order of 800° F. to 1100° F. and is allowed to "soak" in this furnace to thoroughly equalize its temperature. It is then allowed to cool in the furnace to atmospheric temperature. 100

Center pieces of the above steels and thus heat treated have a sorbitic microstructure, being composed mostly of sorbite or sorbite and troostite. The Brinell hardness ranges between 325 and 375. 105

My invention possesses certain distinct advantages over the prior art. In the prior practice of casting the main body of the center piece in such manner as to embed the ends of rail members in the casting, the resulting body cannot be successfully heat treated for the purpose of increasing the physical properties of the center piece, a feature which is so important because of the severe service to which center pieces are exposed. There are 110 several factors which prevent successful heat treatment of such prior structures. One is due to the fact that the composition used in the center piece is different from that used in the rail members secured thereto and the 115 treatment which would be successful with one would not be applicable to the other. Then too, the form and size of such a structure militates against its heat treatment. The larger the body being heat treated the more 120 difficult. But the shape of the structure, with its differently formed part and with parts of radically different dimensions, is an even greater handicap to successful heat treatment. To quench such a structure, with its 125

extended rail members, without distorting the form thereof, is well nigh impossible.

My invention avoids these difficulties. As the center piece is cast separate from the rail members it can be heat treated while still independent of them. It can be given just the heat treatment best adapted to the material of which it is composed. Its weight is much less than that of the combined center piece and rail members and there is not the diversity of form and dimensions with the result that in heat treatment there is much less danger of distortion.

My invention also possesses similar advantages over that type of prior art structure in which the rail members are cast as integral parts with the center piece. Obviously the mass of metal and diversity of shape and dimensions in that type of structure offers the same difficulty in preventing distortion during the heat treatment. Another advantage over this prior type is in the simplification of the foundry practice; obviously it is a much simpler foundry problem to cast the center piece by itself rather than as a structure with integral rail members. Then also obviously much less metal must be handled in the foundry. A further advantage is the economy resulting from limiting the use of special alloy steels to the center piece in contradistinction to the prior practice of casting the rail members integral with the center piece, where the special steels necessary for the center piece must also be used for the rail members. A still further advantage comes from the use with my invention of rolled rail members of the desired size and section which can be selected to match the rails to which they are to be joined. When the rail members are cast integral with the center piece it is usually necessary that the rail members be machined to adapt them to the rails to which they are to be joined.

It will be obvious that a track structure constructed in accordance with my invention presents a minimum sized center portion adapted to be made of a special alloy steel. Its lines are straight which simplifies the pattern, its sections are comparatively uniform which facilitates casting and heat treatment, and being of the same height as the rails gets its support directly from the ties. The center when welded to the rail members provides a structure that is integral without being a one-piece casting that is costly in respect to patterns and more or less uncertain in quality because of its irregular shape and sections. The saving of material and weight over prior methods is also an important factor of economy.

Tests have been made to determine the comparative strength of the welds, with the result that the welds prove to be stronger than the rail members.

Although I have described but one pre-

ferred method of making the welds, it is to be understood that other methods may be employed if desired and while I have shown my invention in but one form it will be obvious to those skilled in the art that it is not so limited, but is susceptible of various other changes and modifications without departing from the spirit thereof, and I desire, therefore, that only such limitations shall be placed thereupon as are imposed by the prior art, or as are specifically set forth in the appended claims.

Having thus described my invention what I claim as new and desire to secure by Letters Patent is:

1. A rail structure comprising a precast metal center-piece of sorbitic microstructure composed of steel containing a moderately high content of silicon and rolled metal rail members integrally secured to the precast center-piece.

2. A rail structure comprising a cast metal center-piece having a sorbitic micro-structure and rolled metal rail members integrally secured thereto.

3. A rail structure comprising a precast, metal center-piece and metal rails integrally secured to the precast center-piece said center-piece having the physical characteristics due to heat treatment.

4. A rail structure comprising a cast metal center-piece having a silicon content of approximately 2% and having a sorbitic micro-structure, and rolled metal members welded thereto.

5. In a railway track structure comprising a cast center having flangeways for wheels in its head portion, rails extending from the ends of said center, the head portion of said rails being in contact only along the upper portions of said ends, and transverse welds uniting the ends of the rails to the center which is of the same height as the rails.

6. In a railway track structure comprising a cast center having base flanges, flangeways for wheels in its head portion, and vertical webs connecting the base flanges and its head portion, rails extending from the ends of said center, the webs and base flanges of said center being spaced from the ends of the rails, and transverse welds uniting the base flanges, webs, and said head portion of the center to the rails, said center being of the same height as the rails and similar in section to the rails.

7. A rail structure comprising a precast metal center-piece sufficiently small in dimensions to be quenched, and rolled metal rail members integrally secured thereto.

In testimony whereof I hereunto affix my signature.

RAYMOND L. GILLISPIE.